

June 30, 1936.

R. W. BEDILION

2,045,576

# METHOD OF AND APPARATUS FOR TREATING METAL CASTINGS

Filed March 9, 1934

4 Sheets-Sheet 1



Fig. 1. INVENTOR  
Robert W. Bedilion  
BY

BY

*Harold Dods*  
ATTORNEY

June 30, 1936.

R. W. BEDILION

2,045,576

METHOD OF AND APPARATUS FOR TREATING METAL CASTINGS

Filed March 9, 1934

4 Sheets-Sheet 2



INVENTOR

*Fig. 2. Robert W. Bedilion*

BY

*Harold Dodd*

ATTORNEY

June 30, 1936.

R. W. BEDILION

2,045,576

METHOD OF AND APPARATUS FOR TREATING METAL CASTINGS

Filed March 9, 1934

4 Sheets-Sheet 3



INVENTOR  
*Robert W. Bedilion*  
BY  
*Frank Dodd*  
ATTORNEY

June 30, 1936.

R. W. BEDILION

2,045,576

METHOD OF AND APPARATUS FOR TREATING METAL CASTINGS

Filed March 9, 1934

4 Sheets-Sheet 4



*Fig. 7.*



*Fig. 8.*

INVENTOR  
*Robert W. Bedilion*  
BY  
*Harold Dodd*  
ATTORNEY

## UNITED STATES PATENT OFFICE

2,045,576

METHOD OF AND APPARATUS FOR  
TREATING METAL CASTINGS

Robert W. Bedilion, United States Navy

Application March 9, 1934, Serial No. 714,741

8 Claims. (Cl. 22—212)

(Granted under the act of March 3, 1883, as  
amended April 30, 1928; 370 O. G. 757)

This invention relates to a method of and means for treating metal castings in the mold while the poured metal is still in the molten condition, to secure a uniform time-rate of cooling of all parts of such casting, thereby eliminating draws and obviating the necessity of the use of chills.

It is the object of this invention to provide electrical means for applying heat to the less massive parts of a metal casting and progressively reducing the heat so applied to cause such less massive parts to cool simultaneously with the heavier portions.

It is a further object to provide means of the type mentioned to maintain the metal of a casting in a liquid state for a sufficient time to permit dross and gases to migrate into the riser and so be removed from the casting.

In the drawings:

20 Figs. 1 and 2 illustrate schematically one apparatus for practicing my present invention;

Fig. 3 is a detail view of one of the magnetic poles;

Fig. 4 shows diagrammatically the application 25 of my invention when the magnetic poles are passed through the walls of the flask;

Fig. 5 is a detail view of a pole extending through the flask and the boot provided to keep the pole free of the mold sand;

30 Fig. 6 illustrates the application of my invention when, for any reason, it is undesirable to make holes through the flask walls;

Fig. 7 shows the positioning of the magnetic poles adjacent the thin parts of a casting in a mold, together with thermo-electric elements embedded in the mold to indicate the temperature adjacent the thin parts of the casting;

Fig. 8 shows the poles provided with auxiliary pole pieces to heat the gate and riser of a casting.

40 Electric heating for furnaces, crucibles, and even for molds in the form of crucibles, has heretofore been known, but so far as I am aware it is entirely novel to utilize induced electric currents in the lighter parts of a casting in the ordinary sand mold to maintain the temperature of those lighter parts substantially equal to that of the more massive parts of the casting.

As shown in Fig. 1, I employ a ring 9, preferably constructed of laminae of soft iron having apertures extending from the inner periphery to the outer periphery thereof through which the laminated poles 10 may be passed. The ring 9 may be either formed of annular laminae or it may be built up of laminated arcuate sections secured together into a continuous body by mem-

bers 11 adjacent the poles 10. As is well shown in Fig. 3, the poles 10 are held in position by plates 12 and 13 which are clamped against the lower and the upper surface thereof by straps 14 and bolts 15. If it is desired to move the poles 5 into or out of ring 9, the nuts 16 on bolts 15 are released, the poles adjusted to the desired position and the nuts again screwed down, thus making any given ring applicable to various sizes of molds. While I have shown in Fig. 1 a ring provided with four poles, it is to be understood that the number thereof may be either greater or less, as occasion or convenience may dictate.

Fixed to ring 9 are a plurality of spools 17 upon which are wound wire coils 18 having a number of turns suitable to produce the desired magnetic flux in the poles 10. The coils 18 are so connected to the current supply that there are formed a plurality of pairs of magnetic poles in each of which pairs the members are of opposite magnetic polarity whereby a magnetic field is set up between the members of each pair. It is readily apparent that when a fluctuating current is supplied to the coils 18 there will be a concomitant fluctuation of the magnetic field between 15 the poles of each pair and therefore currents will be induced in any electrically conducting material within such field and heat will be developed thereby.

The coils 18 are connected to terminal blocks 30 19 which are connected by wires 20 to a load regulator 21 of any well known commercial type. As illustrated, each load regulator 21 has a pilot motor 22 to change the magnetic linkages in the load regulator and thereby vary the output. 35 The load regulators 21 are supplied, through bus bars 23, from a master load regulator 24 having a pilot motor 25, although in some cases the master regulator may preferably be omitted.

Each load regulator 21 is suitably connected, 40 as by wires 26 having an inductive coupling with one of the wires 20, to an ammeter 27 on instrument panel 28 whereby the output of each load regulator may be determined for purposes of control. The pilot motors 22 and 25 are operated by direct current from a supply line 29 and are controlled by reversing switches 30 and 30', respectively, on the instrument panel. The line current and voltage in bus bars 23 are shown by an ammeter 31 and a volt meter 32 suitably connected 50 to the bus bars by pairs of wires 33 and 34, respectively.

A plurality of thermo-couples 35 are embedded in the sand of the mold adjacent the ends of poles 10 and are connected to indicating instru- 55

ments 36 on panel 28 to show the temperatures existing at the places where such thermo-couples are disposed. While there are shown a number of thermo-couples 35 corresponding to the number of poles 10 used, it is to be understood that there will be other thermo-couples positioned to indicate the temperature in the more massive parts of the casting in order that the temperatures may be maintained substantially uniform throughout the body of the casting. As is seen in Figs. 7 and 8, there is a thermo-couple 35 adjacent each part of the casting whereof the temperature is to be controlled by one of the poles 10 and by means of these thermo-couples the operator is apprised when the correct temperature is being maintained or whether it should be increased or reduced, and in accordance with the requirements he will manipulate the switches 30 to augment the current through a coil 18 or 20 reduce the same. The indicating instruments 36 are of a well known type having a settable element to indicate the temperature that should be maintained and it is therefore necessary merely to observe whether the index moved by 25 the current from thermo-couples 35 corresponds with its cooperating set indicating element. A gang shaft 37 for setting simultaneously these elements is indicated on panel 28 and is operable through bevel gears 38 and a suitable hand wheel 30 or other device connected to the bevel gears.

In some cases it may be necessary or desirable to insert the end of the pole 10 within the molding flask to secure less reluctance in the magnetic circuit and a greater field intensity in the metal 35 to be heated. This is accomplished as shown in Fig. 5 wherein the flask is designated by 39 and the metal of the adjacent part of the casting by 40. To permit the molds to be made up on a molding machine and the later insertion of poles 40 10 without disturbing the mold, I provide a boot 41 adapted to fit over the opening in the flask and receive the end of pole 10. The penetration of the pole 10 into the mold may be varied by using any necessary number of spacers 42 between 45 the boot and the flask. The general arrangement of the equipment when so used is shown in Fig. 4 wherein the same reference characters denote the same parts as in Fig. 5. In Fig. 6 the mold is not penetrated by the poles.

Fig. 7 shows the ring and poles supported upon legs 43 to position the poles properly with respect to a tall casting. In cases where it may be necessary to heat a relatively wide belt, the rings with their poles may be stacked one upon the other, 55 bosses 44 being provided upon the upper surfaces of the rings to position the legs 43 which may be pipes adapted to fit over such bosses.

In Fig. 8 a disk-like casting 45, together with the gate and riser, are heated by means of the 60 poles 10 and auxiliary laminated pole pieces 46 which spread the magnetic field over a greater area.

After the mold is made, the flask is positioned within the ring 9 to dispose the poles 10 opposite 65 the lighter parts of the casting to secure localized heating of such parts. While for the purpose of simplicity of illustration I have shown the poles supported in substantially a common annular zone, the ring 9 may be laterally off-set in any 70 manner to apply the heat as required to any given casting, or the poles may be connected together in various other ways to complete the magnetic circuit. When the casting has been poured it will frequently be found desirable to apply heat by my 75 apparatus to keep the metal fluid until the dross

and gases have risen to the upper portion of the metal, which will result in much stronger and sounder castings. The casting is then allowed to begin to cool; meanwhile, the operator keeps careful check upon the temperatures of the various parts of the casting. When it is observed that one part is cooling more rapidly than some other part, heat is applied to maintain the temperature of the more rapidly cooling part, and the heat so applied is progressively reduced to 10 cause all portions of the casting to cool simultaneously and at substantially the same time-rate, whereby there will be no tendency to the development of draws due to a cool part contracting away from a still molten part. It is thus apparent that with my method it is unnecessary to use chills to hasten the cooling of the heavier parts of the casting, as is common practice. 15

Another advantage of my method is that castings of any size may be poured successfully. As practiced heretofore it has been necessary to make one pour of all the metal in a casting, but by the use of my apparatus the metal in the mold may be kept in a highly fluid state until any required number of pours may have been made to secure a casting of any desired size. 20

The invention described herein may be manufactured and used by or for the Government of the United States of America for governmental 30 purposes, without the payment of any royalties thereon.

I claim:

1. In combination, a laminated supporting ring of magnetic material adapted to be disposed around a mold having in it a casting cavity, said ring having openings extending from the outer periphery to the inner periphery thereof, an inductive coil mounted on the said inner periphery with a central passage in registry with each of the aforesaid openings, a laminated pole extending through each of the said openings and the adjacent coil, with the end of the pole positioned to lie adjacent a predetermined region of said cavity, said coils being connected to provide pairs of poles of opposite magnetic polarity, and means to indicate the temperature adjacent each pole. 35

2. In combination, a supporting ring of magnetic material adapted to be disposed around a mold having in it a casting cavity, said ring having openings extending from the outer periphery to the inner periphery thereof, an inductive coil mounted on the said inner periphery with a central passage in registry with each of the aforesaid openings, a pole extending through each of said openings and the adjacent coil with the end of the pole positioned to lie adjacent a predetermined region of said cavity, means to supply current to each coil, said coils being connected to provide pairs of poles of opposite magnetic polarity, and means to indicate the temperature adjacent each pole. 50

3. In combination, a laminated supporting ring of magnetic material adapted to be disposed around a mold having in it a casting cavity, said ring having openings extending from the outer periphery to the inner periphery thereof, an inductive coil mounted on said inner periphery with a central passage in registry with each of the aforesaid openings, a laminated pole extending through each of said openings and the adjacent coil with the end of the pole positioned to lie adjacent a predetermined region of said cavity, means to supply current to each coil, said coils being connected to provide pairs of poles of opposite magnetic 65

posite magnetic polarity, thermo-electric means to indicate the temperature adjacent each of said poles, said last means comprising an element to indicate the temperature it is desired to maintain adjacent each pole, and means to control the flow of current to each coil individually.

4. The combination with a molding flask having a plurality of openings through the sides thereof, of a hollow member adjacent each of said openings, said members each having an open end in registry with its respective opening and a closed end spaced therefrom to lie immediately adjacent a predetermined region of a casting cavity in said flask, a pole piece extending into each of said members substantially to said closed end, an inductive coil disposed around a portion of each pole piece, means to supply alternating current to each of said coils to provide pairs of poles of opposite magnetic polarity, and means to control the current supply to each of said coils individually.

5. The combination with a molding flask having a plurality of openings through the sides thereof, of a hollow member adjacent each of said openings, said members each having an open end in registry with its respective opening and a closed end spaced therefrom to lie immediately adjacent a predetermined region of a casting cavity in said flask, a pole piece extending into each of said members substantially to said closed end, an inductive coil disposed around a portion of each pole piece, means to supply alternating current to each of said coils to provide pairs of poles of opposite magnetic polarity, means to control the supply of current to each of said coils individually, a thermo-couple disposed adjacent

each of said poles, and temperature indicating means actuated by the thermo-electric current from each of said coils.

6. The method of making large castings that require a quantity of metal greater than one pour, which comprises making a pour, setting up in the poured metal fluctuating magnetic fields to induce electric currents to maintain the temperature of the poured metal until a subsequent pour and so continuing until the required quantity has been poured, thereafter maintaining the said fields in the less massive portions only of the casting and progressively reducing the strength of the said maintained fields to cause all parts of the casting to cool simultaneously. 15

7. The method of making large castings that require a quantity of metal greater than one pour, which comprises making a pour, setting up in the poured metal fluctuating magnetic fields to induce electric currents to maintain the temperature of the poured metal until a subsequent pour and so continuing until the required quantity has been poured, adjusting the heating effect to maintain the temperature of the less massive portions, and then permitting the casting to cool. 20

8. The combination with a molding flask adapted to contain a mold having in it a cavity, said flask having a plurality of openings through the sides thereof, of a hollow member adjacent each of said openings, said members each having an open end in registry with its respective opening in the flask and a closed end spaced therefrom within the flask adjacent the position of said cavity.

ROBERT W. BEDILION. 35